

# UNITED STATES PATENT OFFICE.

FRITZ PFLEUMER, OF DRESDEN, GERMANY, ASSIGNOR TO PFLEUMATIC SYNDICATE LIMITED, OF LONDON, ENGLAND, A CORPORATION OF GREAT BRITAIN.

MANUFACTURE OF AN ELASTIC CELLULAR OR SPONGY MATERIAL FOR USE AS A FILLING FOR VEHICLE-TIRES, CUSHIONS, BUFFERS, UPHOLSTERY, AND THE LIKE.

932,318.

Specification of Letters Patent. Patented Aug. 24, 1909.

No Drawing.

Application filed April 24, 1908. Serial No. 429,054.

To all whom it may concern:

Be it known that I, FRITZ PFLEUMER, a subject of the Emperor of Austria-Hungary, residing at Dresden, Germany, have invented 5 certain new and useful Improvements in the manufacture of an elastic cellular or spongy material for use as a filling for vehicle-tires, cushions, buffers, upholstery, and the like, of which the following is a specification.

This invention relates to improvements in the manufacture of an elastic cellular or spongy material for use as an elastic filling for hollow vehicle-tires, cushions, seats, mat- 15 tresses, balls, buffers, elastic saddles, ship's fenders, upholstery, and the like.

The improved process depends on the well known fact that sheets of gelatin, which have been left for some days in a solution 20 of pyrogallol, with access of air, are quite insoluble after drying. This fact is however not directly available for the purpose in view, as one cannot leave the mass of glycerin and gelatin in a pyrogallol-solution 25 to soak and then dry it. The pyrogallol must rather be added in aqueous or alcoholic solution to the material and the various solutions employed for this purpose should not form too great a proportion of the mass of 30 glycerin and gelatin as the latter would then become too thin or fluid.

In place of pyrogallol one can employ other substances, such as metaphenylenediamin, paraphenylenediamin, and particu- 35 larly those of the phenol-group, for example hydroquinone, pyrocatechin, paramidopheno- 40 nol, diamidophenol chlorid, diamidoresorci- nol chlorid, metoquinone (a mixture of 10 parts metol with 3 parts of quinol or hydro- 45 quinone) "adurol" (mono-chlor-hydroquinone or mono-brom-hydroquinone), "eikogen" (sodium amido- $\beta$ -naphthol- $\beta$ -sulfonate), "metol" (para-methyl-amido- meta-cresol-sulfate), also gallic acid, tannic 50 acid,  $\alpha$  and  $\beta$  naphthol, resorcinol, phloroglucinol, dioxynaphthalene. Moreover, two or more of these substances can be employed together. In this way, one can for example regulate the rate of tanning by mixing in 55 suitable proportions, an actively tanning and a feebly tanning phenol and allowing them to act together. The actively tanning sub- 60 stance will react first, but the action of the feebly tanning medium will continue for a

longer time. The chemical action of these 55 substances on glycerin or glue depends upon the fact that these tanning media take oxygen from the air and transfer it to the gelatin or glue and thereby render the latter substances insoluble. The gelatin and glue are 60 more difficult to dissolve in water, in proportion as more oxygen is taken from the air and transferred thereto. This effect can be increased to such a degree that the gelatin (glue) remains perfectly insoluble even if 65 allowed to lie for hours in boiling water.

The process is carried into practice in the following manner: 6 kilograms of gelatin powder are steeped in 9 kilograms of glycerin until the mass is quite stiff. These proportions by weight can be altered within cer- 70 tain limits, for example, 4:11, 5:12, 7:8 kilogr., according to the consistency or de- 75 gree of toughness or viscosity desired and the quality of the material employed. But if, for example, gelatin of inferior quality is employed, then almost as much gelatin as glycerin can be employed; when using glue one can take more glue than glycerin in order to attain the same effect as when em- 80 ploying the best gelatin under the above conditions. This steeped mass is next heated in a boiler or other suitable vessel to a tem- 85 perature of about 158° F. In order to enable this temperature to be maintained per- 90 fectly uniform, the boiler is stood in a water- bath, this being effected by placing the boiler inside another vessel. The space left be- 95 tween the two vessels is filled with water, the temperature of which can be checked by means of a thermometer. When the mass is heated through sufficiently, it is stirred by means of a stirrer for about 1 to 2 hours. By this means, the mass becomes homo- 100 geneous, i. e. of perfectly uniform toughness and consistency in all parts, which is es- 105 pecially important in order to obtain an ample formation of bubbles, cells or foam.

The formation of the gelatin into cells or foam can be considerably promoted if very 100 finely pulverized material, such for example, as finely powdered and sifted oxid of zinc is added to it and stirred in uniformly with the stirrer. This powder does not act chem- 105 ically, but only physically by affording points for the development of the vapor phase. By this means it results that the formation of bubbles or cells begins even in

the stirring vessel, which action starts the formation of bubbles or cells, which is to be effected under pressure, considerably more quickly than when the mass is not previously stirred. For the above given quantity of 15 kilograms of material, about 250 grams of finely powdered zinc oxid are taken. Also finely divided insoluble substances in suspension, *e. g.* flowers of sulfur suspended in 10 water, are suitable for this purpose.

From the stirring boiler or vessel, the material comes into the foam-beating boiler, in which it is to be turned into foam. This must be so arranged, that a high pressure 15 can be produced therein, for the higher the pressures under which the mass is beaten, the more aerated and also the lighter will the material be after cooling. A pressure of from 20 to 40 atmospheres is preferably employed (295 to 590 pounds per square inch). 20 However this process of producing bubbles or foam is not the object of the present invention. It is already dealt with in the specification of my former Letters Patent No. 25 851,960. Into this 15 kilograms of material, when it is already in the foam-beating-boiler, the tanning substance is stirred. According to the degree of tanning desired, 2 to 100 grams of pyrogallol may be employed, 30 more or less. Preferably however, when working at a temperature of the material of 158° F. and a pressure of 30 atmospheres (440 pounds per square inch), 20 grams of pyrogallol are employed. This quantity of 35 pyrogallol can be dissolved in any desired amount of water or of alcohol or other solvent of any strength, and the solution then stirred into the mass. The quantity of this solution taken should not be too great in 40 order not to dilute the mass too much and to avoid hydrolysis or hydrolytic cleavage of the gelatin; on the other hand it must be sufficient for the tanning medium to be distributed well throughout all parts of the 45 mass. For the above mentioned quantity of 20 grams of pyrogallol one takes about 100 grams of water. As however the mixture of glycerin and gelatin is employed in hot liquid condition at a temperature of about 50 158° F. and the heat acts to accelerate the tanning process considerably, special precautionary measures must be taken, so that the tanning medium after the mixing does not act too quickly, for after the mixing-in 55 of the tanning medium, the mass is to be turned into foam by means of a beating-apparatus. This beating operation lasts from 2 to 5 minutes, assuming that the formation of the foam was previously started 60 by the stirrer. If at this time, the tanning medium acts too quickly, the consistency or viscosity of the mass becomes too great. This would be very unfavorable for the formation of foam, as the formation of foam 65 proceeds best at a definite consistency or

viscosity. The pyrogallol, dissolved in water can therefore be advantageously introduced into the mass by means of a powdery material of great absorbent power acting as a restrainer. Infusorial earth or kieselguhr, 70 which is specially adapted for this purpose, is preferably employed. This powder, saturated with the solution, is stirred into the mass and during the beating gives up the tanning medium to the mass, so that the 75 tanning only begins when the greater part of the foam has already been formed.

In cases where the zinc oxid or like material is not used, the following proportions may also be employed, the process being 80 otherwise carried into practice as hereinbefore described, *viz.*:

|                  |     |                  |
|------------------|-----|------------------|
| Powdered gelatin | 360 | parts by weight. |
| Liquid glycerin  | 620 | " "              |
| Pyrogallol       | 4   | " "              |
| Infusorial earth | 8   | " "              |
| Water            | 8   | " "              |

The tanning action can be promoted by mixing alkalies or bromin with the tanning medium. These means cause the tanning action to take place at a higher rate. They can be employed with those phenols which tan very slowly, but their employment is excluded in the case of those that 90 act very quickly, as for example pyrogallol. The tanning action can also be promoted, without increasing the rate at which the tanning progresses, by raising the oxygen-content of the air which is forced into the beating boiler before the beginning of the beating; in this case however the amount of tanning medium is reduced for the tanning action obviously only lasts so long as a sufficient quantity of oxygen is present in the 100 compressed air in the foam. As soon as this is absorbed, the further progress of the tanning stops.

This process can be carried into practice as follows:—First of all pure oxygen is 110 forced into the foam-beating boiler, after the latter has been closed, until the pressure rises to  $7\frac{1}{2}$  atmospheres (110 pounds per square inch) and after this ordinary air is forced in until the pressure rises to 30 115 atmospheres (440 pounds per square inch). Then the gaseous mixture in the boiler contains about twice as much oxygen as ordinary air of the same pressure, under which conditions one takes only 10 grams of pyrogallol instead of 20 grams. Then, so long as 120 the mass is hot, the subsequent tanning action lasts much longer than when employing ordinary air, since the supply of oxygen in the beaten-in gaseous mixture lasts much longer than with ordinary air. The rate at which the tanning takes place, which rate would increase if one employed the same quantity of pyrogallol as when ordinary air 125 is employed, is thus equalized, when using 130

air enriched by oxygen, by reducing the amount of tanning medium.

The residue of oxygen in the bubbles can be almost completely utilized if the bodies, 5 into which the beaten material is introduced, *e. g.*, tires, cushions, balls, etc., after they have been filled, are heated for some hours to about 158° F.

What I claim is:—

10 1. A process for the manufacture of an elastic cellular or spongy material for filling tires and for like purposes, consisting in soaking gelatin in glycerin, heating the mixture, adding thereto a tanning material dissolved in a liquid which is carried by an absorbent neutral powder, and beating the mixture into foam with a gas containing oxygen.

20 2. A process for the manufacture of an elastic cellular or spongy material for filling tires and for like purposes, consisting in soaking gelatin in glycerin, heating the mixture, adding thereto a plurality of tanning media of different rates of tanning dissolved 25 in a liquid, and beating the mixture into foam with a gas containing oxygen.

30 3. A process for the manufacture of an elastic cellular or spongy material for filling tires and for like purposes, consisting in soaking gelatin in glycerin, heating the mixture, adding thereto a very finely powdered material, stirring the mixture, adding a tanning material dissolved in a liquid, and beating the mixture into foam with a gas containing 35 oxygen.

40 4. A process for the manufacture of an elastic cellular or spongy material for filling tires and for like purposes, consisting in soaking gelatin in glycerin, heating the mixture, adding thereto a tanning substance and a substance for accelerating the action of said tanning material, said substances being held in solution in a liquid, and beating the mixture into foam with a gas containing 45 oxygen.

50 5. A process for the manufacture of an elastic cellular or spongy material for filling tires and for like purposes, consisting in soaking gelatin in glycerin, heating the mixture, adding thereto a tanning material dissolved in a liquid, and beating the mixture into foam with a gas containing oxygen.

55 6. A process for the manufacture of an elastic cellular or spongy material for filling tires and for like purposes, consisting in producing a homogeneous mixture of gelatin and glycerin, heating the mixture, adding thereto tanning material dissolved in a liquid which is carried by an absorbent 60 neutral powder, beating the mixture into

foam with a gas containing oxygen, introducing said foam into a hollow receptacle, *e. g.* a vehicle tire, and afterward subjecting said foam in said receptacle to an elevated temperature for a suitable time, substantially as described.

65 7. A process for the manufacture of an elastic cellular or spongy material for filling tires and for like purposes, consisting in producing a homogeneous solution of gelatin in glycerin, adding a finely pulverized material thereto, stirring the mixture in a heated condition, adding thereto tanning material dissolved in a liquid which is absorbed by a neutral powdery material, and 70 beating the mixture into a foam with atmospheric air under pressure.

75 8. A process for the manufacture of an elastic cellular or spongy material for filling tires and for like purposes, consisting in soaking powdered gelatin in glycerin, heating the mixture, stirring the mixture, adding powdered zinc oxid thereto, adding thereto tanning material dissolved in a liquid which is absorbed by infusorial earth, and beating 80 the mixture into a foam with atmospheric air under pressure.

85 9. A process for the manufacture of an elastic cellular or spongy material for filling tires and for like purposes, consisting in soaking gelatin in glycerin, heating the mixture, beating the same into foam with compressed air, adding to said mixture a solution of pyrogallop and a restrainer, and stirring the 90 said mixture.

95 10. A process for the manufacture of an elastic cellular or spongy material for filling tires and for like purposes, consisting in mixing together gelatin, glycerin and a finely powdered material at a high temperature, stirring the mixture, adding a tanning material and a restrainer, and beating the resultant mixture into a foam with gas in the presence 100 of an oxidizing medium.

105 11. A process for the manufacture of an elastic cellular or spongy material for filling tires and for like purposes, consisting in soaking gelatin in glycerin, heating the mixture, beating the same into foam with a gas, adding to said mixture a solution of pyrogallop and a restrainer, and stirring the resultant mixture with an oxidizing medium.

In testimony whereof I have hereunto set my hand in presence of two subscribing witnesses.

FRITZ PFLEUMER.

Witnesses:

PAUL ARRAS,  
ROBERT J. CALDWELL.